

No. 835,148.

PATENTED NOV. 6, 1906.

B. C. WHITE.  
MANUFACTURE OF GLASS PLATES.

APPLICATION FILED JAN. 8, 1903

3 SHEETS—SHEET 1.



No. 835,148.

PATENTED NOV. 6, 1906.

B. C. WHITE.

MANUFACTURE OF GLASS PLATES.

APPLICATION FILED JAN. 8, 1906.

3 SHEETS—SHEET 2.



WITNESSES:

*John C. White*  
*Herbert Bradley*

Bruce C. White **INVENTOR**  
by Christy and Christy,  
Atty's.

No. 835,148.

PATENTED NOV. 6, 1906.

B. C. WHITE.

MANUFACTURE OF GLASS PLATES.

APPLICATION FILED JAN. 8, 1906.

3 SHEETS—SHEET 3.



WITNESSES:

*J. H. Burgess*  
*Herbert O. Bradley*

INVENTOR  
*Bruce C. White*  
*by Christy and Christy,*  
*Atty's*

# UNITED STATES PATENT OFFICE.

BRUCE CLARK WHITE, OF CHICAGO, ILLINOIS.

## MANUFACTURE OF GLASS PLATES.

No. 835,148.

Specification of Letters Patent.

Patented Nov. 6, 1906.

Application filed January 8, 1906. Serial No. 295,108.

*To all whom it may concern:*

Be it known that I, BRUCE CLARK WHITE, a citizen of the United States, formerly residing at Mosgrove, Pennsylvania, but now residing at Chicago, in the county of Cook and State of Illinois, have invented or discovered certain new and useful Improvements in Manufacture of Glass Plates, of which improvements the following is a specification.

10 In Letters Patent No. 805,610, granted to me November 28, 1905, I have described and claimed an improvement in the manufacture of glass plates which consisted, generally stated, in forming a portion of sheet and then forming the remaining portion on the portion first formed. In the specific method and apparatus disclosed in said patent the portion first formed is reduced to shape and thickness approximately and then distributed 15 along or deposited on a bed or table, and the remaining portion of glass is reduced to shape and approximate thickness and distributed along or deposited on the portion first formed.

20 The invention described herein relates to certain additional or further improvements in that method broadly claimed in said patent; and it consists, generally stated, in spreading a portion of a mass of glass along a bed or table and then spreading the remaining portion of the mass in a reverse direction on and along the portion first reduced. The invention is hereinafter more fully described and claimed.

25 In the accompanying drawings, forming a part of this specification, Figure 1 is a top plan view of a form of mechanism adapted to the practice of my invention. Fig. 2 is a side elevation of the same. Figs. 3, 4, and 5 show in section the parts directly operating on the glass and illustrate different stages in the formation of the plates. Figs. 6 and 7 are sectional detail views illustrating a construction for determining the desired relative 30 position of the spreading-rolls and table. Figs. 8 and 9 are similar views illustrating a modification of the construction shown in Figs. 5 and 6. Figs. 10 and 11 are plan and side elevation, respectively, of another form 35 of apparatus for the practice of my improved method. Fig. 12 is a sectional detail view illustrating a means for spacing the rolls and table.

In the practice of my invention the proper spacing of the spreading-rolls and the relative

to the table can be accomplished in many ways. A desirable construction for that purpose consists in securing to or forming on the table two lines of rails 4 and 5, the rails 5 projecting a greater height from the surface of the table than the rails 4. While not essential, it is preferred that the rolls should be made of the same or approximately the same length and that the rails 5 should have their supporting-surfaces above and as nearly as practicable in line with the corresponding surfaces of the rails 4, so as to permit of the utilization of a maximum amount of the surface of the table for forming purposes. In order to permit of the roll 1 resting on the rails 4, grooves 6 are cut in the roll for the reception of the rail 5, as clearly shown in Figs. 4 and 5. The distance the rails project above the surface of the table determines the thickness of the portion of the sheet first formed, while the thickness of the portion of the sheet formed on the first portion is determined by the height of the surface of rail 5 above the bed or table.

Where a side delivery of the finished plate 40 is desired, the roll supporting and spacing rails are omitted, and the rolls are provided with collars 25, which are loosely mounted in grooves in the rolls. These collars roll along the table, and by properly proportioning the 45 thicknesses of the collars the proper spacing of the rolls relative to the table is attained. As the collars are loose on the rolls, the latter can slip therein, thus avoiding a rubbing movement of the rolls on the glass.

50 In forming "plates," as I prefer to term the completed article, a sufficient quantity of glass to produce the two portions of the sheet composing the finished plate is poured onto the table in front of the roll 1, which is 55 then caused to roll forward along the table and spread a portion of the glass over the surface of the table. After the first portion of the sheet is formed, the roll 2 is brought 60 into operation, moving along the table in a 65 direction the reverse of the operative movement of the roll 1, which is returned to its initial position, so as not to interfere with the operation of the roll 2. As the roll 2 moves along over the table it spreads the remaining 70 portion of the glass over the surface of the glass spread by the roll 1. The pressure exerted by the roll 2 on the glass spread or distributed thereby forces it tightly down on the portion of the sheet first formed. If it is 75

desired to incorporate a metallic web in the plate formed as described, it is placed on the portion of the sheet formed forward or operative movement of the roll 1 and before said roll is returned to its initial position, so that such return movement may be utilized to embed the fabric or wire mesh in the first-formed portion of the sheet, and thus providing a smooth surface on which to spread the remaining portion of the glass.

While the rolls 1 and 2 may be caused to traverse the table successively and independently of each other, it is preferred that they should be coupled together so as to traverse the table simultaneously in both directions. The rolls can be coupled by any suitable means—as, for example, by the bars 6, having collars 7, fitting loosely over the trunnions 8 on the ends of the rolls, as shown in Figs. 1 and 2. When the rolls are thus coupled, the glass is poured onto the table between the rolls, which are then caused to move forward and back over the table, or the latter is given a similar movement under the rolls. During the forward movement of the rolls or table one of the former will act to spread a portion of the glass on the table, and during the backward movement the other roll will act to spread the remaining portion of the glass over the surface of the portion first spread.

Any suitable means may be employed for causing the forward and return movements of the rolls—such, for example, as that shown in Figs. 1 and 2. The rolls 1 and 2 are provided at their ends with sprocket-wheels 10, having their pitch-diameters equal to the diameters of the rolls, and sprocket-wheels 11 and 12 are secured to shafts 13 and 14, mounted in suitable bearings at the respective ends of the table. Chains 15, having one end secured to anchors 16 at one of the tables, pass over the sprocket-wheels on one of the rolls, back over the sprocket-wheels at the end of the table where the chains are anchored, forward over the sprocket-wheels at the opposite end of the table, back around the sprocket-wheels on roll 2, and then forward to anchors 17. While power may be applied to one of the rolls or to the shaft, it can be more conveniently applied to the shaft, as 13. As this shaft is rotated the rolls are similarly rotated by the chains and caused to roll toward the shaft 13. When the shaft is rotated in the opposite direction, the rotation of the rolls is reversed, and they will roll toward the opposite end of the table.

While not necessary, it is preferred to provide a support for the metal fabric which is to be incorporated in the plate. Such support is conveniently formed by extending the coupling-bars 6 and connecting such extensions by a cross-bar 18, to which is secured a fabric-supporting plate 19, arranged in a

plane tangential or approximately tangential to the roll 1 adjacent to its line of contact with the formed sheet, so that such fabric will readily feed down under the roll 1 during its return movement.

As shown in Figs. 10 and 11, the rolls 1 and 2 may be mounted in stationary bearings 20 and the table 3 mounted on wheels 21 to permit of its being reciprocated forward and back under the rolls. In this construction the rolls are driven by the table, which can be reciprocated by any suitable means. In order to rotate the rolls, toothed wheels 22 are secured thereto. Racks 23 are secured to or formed on the table.

It is characteristic of my improved method that the fabric is not applied to the glass until it has become somewhat hardened and stiff, thus preventing any distortion of the glass, which being embedded in the portion first formed, and therefore somewhat stiff but yielding, will hold the fabric in place while the remaining portion of the glass is being spread over it.

I claim herein as my invention—

1. The method herein described of forming glass plates consisting in placing a mass of glass on a bed or table, spreading a portion of said glass in one direction in the form of a sheet and spreading another portion of the glass in the opposite direction over and upon the portion first spread.

2. The method herein described of forming glass plates consisting in placing a mass of glass on a bed or table, spreading a portion of said glass in one direction in the form of a sheet and spreading the remaining portion of the glass in the opposite direction over and upon the portion first spread.

3. The method herein described of making glass plates which consists in depositing a mass of glass upon a table, spreading a portion of said glass in one direction into a sheet form, placing a web or fabric upon the portion spread and spreading another portion of the glass in the opposite direction over and upon the fabric and the portion first spread.

4. The method herein described of forming glass plates consisting in placing a mass of glass upon a bed or table, spreading a portion of said glass in one direction into sheet form, embedding a fabric or web in the surface of the portion spread and spreading another portion of the glass in the opposite direction over and upon the portion first spread.

5. The method herein described of making glass plates consisting in placing a mass of glass upon a table between two rollers, moving one of the rollers along the table and spreading a portion of such mass of glass into sheet form and then moving the other roller in the opposite direction and thereby rolling another portion of the mass over and upon the portion first spread.

6. The method herein described of making

glass plates which consists in depositing a mass of glass upon a table between two rollers, moving said rollers along the table and thereby spreading a portion of the glass into sheet form, reversing the direction of movement of the rollers, introducing a fabric or web between the portion spread and the roller effecting such spreading operation and by the action of the other roller spreading

the remaining portion of the glass onto the portion first spread.

In testimony whereof I have hereunto set my hand.

BRUCE CLARK WHITE.

Witnesses:

CHARLES BARNETT,  
J. C. MCCORMICK, JR.